

Sept. 17, 1929.

E. C. DEARDEN

1,728,398

MANUFACTURE OF MOSAIC FABRICS

Filed Sept. 22, 1927



Fig. 1.



Fig. 2.



Fig. 3.

Fig. 4. *Inventor:*  
Edward C. Dearden,

*By S. S. Dearden*  
*Attorney*

## UNITED STATES PATENT OFFICE

EDWARD C. DEARDEN, OF MERION, PENNSYLVANIA, ASSIGNOR TO THE GEO. W. BLABON COMPANY, OF PHILADELPHIA, PENNSYLVANIA, A CORPORATION OF PENNSYLVANIA

## MANUFACTURE OF MOSAIC FABRICS

Application filed September 22, 1927. Serial No. 221,221.

My invention is an improvement in the manufacture of flexible mosaic fabrics designed to provide a floor covering or the like having portions of its surface in relief to accentuate the figures of its pattern and to interrupt the light reflecting surface thereof; such projections of figures or borders resulting from differences in the expansibility of the compositions from which the tesserae comprised in the pattern are made.

By my improvements, I am enabled to produce a flexible mosaic fabric having a surface in relief without embossing or indenting the surface, and am also enabled to use for the different tesserae compositions of the same or similar ingredients and proportions of ingredients, and to deposit the linoleum composition initially upon the backing in layers of uniform thickness.

My present invention is based primarily upon my discovery and utilization of the fact that linoleum compositions vary in resiliency and expansibility with age, and by suitably aging the composition designed to form the projecting tesserae I am able to secure a desired excess expansion of the tesserae formed therefrom after the product has been compacted in a heated hydraulic press or otherwise. This unequal expansion of the tesserae results in an impressed effect notwithstanding the fact that the sheet prior to pressing may be initially of uniform thickness and may be pressed by plates or rollers having smooth plane surfaces.

The extent of the differences in the age of the different compositions used in making mosaic fabrics are dependent upon the degree of inequality of the expansion of the tesserae desired and to some degree upon the constituents and proportions of the composition. I have found that a usual composition of oxidized linseed oil, ground cork, wood flour, and pigment is given sufficient additional expansibility by aging for a week to form a satisfactory ridge or bead projecting beyond the surface of tesserae formed of freshly made linoleum composition of like ingredients and proportions after both have been compacted by passing through a steam heated hydraulic press. Instead of aging

the composition itself, I may, of course, age the oxidized linseed oil alone, or use another binder whose expansibility after compression is increased by aging.

Steps involved in the preferred practice of my invention, and a product resulting therefrom, are graphically illustrated in the accompanying drawings, in which Fig. 1 is a fragmentary top plan view of tesserae of granulated linoleum composition loosely deposited upon a backing to form a pattern of tiles separated by mortar joints; Fig. 2 illustrates a cross sectional view on the line 2—2 of Fig. 1 and also shows diagrammatically the bed and top plate of a hydraulic press for compacting the loose granular material; Fig. 3 is a fragmentary top plan view of the product resulting from compacting the material shown in Figs. 1 and 2; and Fig. 4 is a transverse sectional view on the line 3—3 of Fig. 3.

In the preferred practice of my invention, comparatively fresh granulated linoleum compositions, differing in color or shade are deposited on a backing 1 to form contrasting plaques or tesserae 2 and 3 which are spaced from one another to provide for the deposit of strips or tesserae 4 composed of granulated linoleum composition which has been aged to increase its resiliency or expansibility.

The deposit of the loose granular composition may be conveniently effected by the use of a plurality of stencils or templates having apertures with contours like that of the various tesserae to be produced. Suitable composition is deposited through the apertures of each stencil and leveled off before the stencil is raised to permit the movement of the backing with the composition thereon. The backing is moved step by step from one to the other of the stencils and receives deposits of the various compositions until the design is completed.

Preferably the stencils are positioned at equal distances above the backing during the deposit of the compositions so that the deposits are of equal thickness or height when moved onto the bed 5 of a steam heated hydraulic press having a top plate or head 6. The descent of the top plate compacts all of

- the compositions to approximately one-third their initial thickness. After a suitable interval the pressure of the press is released. The compacted compositions 2 and 3 thereupon expand slightly, but the aged composition 4 expands considerably more than the compositions 2 and 3 so as to produce ridges or beads 4' forming a projecting grid above the general surface level.
- 10 The interlacing of the granules at the side edges of the tesserae 4 with the granules at the side edges of the tesserae 2 and 3 tend to restrain the expansion of the tesserae 4 immediately adjacent the edges thereof so that 15 the ridges 4' are slightly higher at the center than at the edges, which latter verge without any sharp angles or breaks into the surface of the tesserae 2 and 3. Other designs, not involving the simulation of tiles, 20 may of course be made in accordance with my invention by forming tesserae that can project above the surface from a more resilient composition than the other tesserae. Or if it is desired that tesserae such as 2 and 3 25 be spaced by depressions or grooves instead of by ridges or beads, this may be effected by using an "aged" composition for the tesserae 2 and 3 and a fresher composition for the strips 4.
- 30 While I prefer that plastic compositions involved in my invention be composed of oxidized linseed oil, granulated cork, wood flour, gums and pigment, other binders rendered more resilient or expandable by aging 35 or oxidation may be used, and fillers such as ground leather or asbestos may be incorporated in the composition in substitution for or in addition to those preferred. All such compositions are intended to be 40 embraced within the term "linoleum composition" as used in the claims, whether or not such composition actually contains any linseed oil or cork. The fillers are generally unaffected by aging, but usually combine 45 more readily and intimately with the binder prior to the final aging and oxidation for increasing the resilience or expansion, than after such final aging. The claims are intended to cover the process and product 50 regardless of whether the filler is incorporated in the binder before or after final aging. The backing may be of burlap, asphaltum treated felt, paper or other suitable sheet material.
- 55 Having described my invention, I claim:
1. A mosaic fabric comprising tesserae composed of inlays of plastic compositions unequally aged to produce unequal elasticities in the tesserae.
- 60 2. A mosaic fabric comprising tesserae composed of inlays of plastic compositions containing a binder rendered resilient by oxidation, such compositions containing binders unequally oxidized.
- 65 3. A mosaic fabric comprising a backing

having attached thereto plastic tesserae composed of granular particles and an expandible binder, said tesserae being unequally aged and the binders thereof of unequal elasticities.

4. A mosaic fabric comprising tesserae of linoleum compositions simulating tile or stone and mortar tesserae simulating mortar joints between said tesserae first named, tesserae aforesaid being formed of composition of greater age than the composition composing other tesserae aforesaid and projecting above the latter.

5. The method of making mosaic fabrics which comprises forming tesserae thereof of compositions whose resilience is increased by age, the compositions forming certain tesserae being aged longer than the compositions forming other tesserae, and compacting the tesserae.

6. The method of making mosaic fabrics which comprises unequally aging linoleum compositions, depositing upon a backing tesserae formed of differently aged compositions, and compacting and uniting such tesserae by pressure.

7. The method of making mosaic fabrics which comprises depositing on a backing spaced tesserae of linoleum compositions filling the spaces between said tesserae with linoleum composition of greater age than said composition first named, and compacting and uniting said tesserae and filler by pressure.

8. The method of making mosaic fabrics which comprises depositing granulated linoleum composition upon a backing through apertures in a stencil having the contours of patterned figures, depositing contrasting linoleum composition on said backing through apertures in a second stencil having the contours of complementary patterned figures, depositing on said backing granulated linoleum composition through apertures having contour of spaces between figures aforesaid, said composition last named being aged longer than the remaining compositions, compacting and uniting said composition by pressure, and releasing said pressure, said composition last named expanding more than said composition first named.

In witness whereof I have hereunto set my name this 16th day of September, 1927.

EDWARD C. DEARDEN.

120

125

130